

# United States Patent

Kubotera et al.

[15] 3,657,022

[45] Apr. 18, 1972

[54] PROCESS FOR THE MANUFACTURE  
OF COLD-ROLLED STEEL STRIP WITH  
SUPERIOR MECHANICAL  
WORKABILITY, ESPECIALLY DEEP  
FORMING PROPERTIES

[72] Inventors: Haruo Kubotera; Kazuhide Nakaoka;  
Kaoru Watanabe; Teruhisa Tanaka, all of  
Kawasaki, Japan

[73] Assignee: Nippon Kokan Kabushiki Kaisha, Tokyo,  
Japan

[22] Filed: Nov. 12, 1969

[21] Appl. No.: 871,559

## Related U.S. Application Data

[63] Continuation of Ser. No. 567,334, July 20, 1966,  
abandoned.

## Foreign Application Priority Data

Aug. 10, 1965 Japan.....40/48225

[52] U.S. Cl.....148/2, 148/12.1, 148/16

[51] Int. Cl.....C21d 1/74

[58] Field of Search.....148/2, 3, 12.1, 16, 39, 134

[56]

## References Cited

### UNITED STATES PATENTS

|           |         |                       |           |
|-----------|---------|-----------------------|-----------|
| 3,281,286 | 10/1966 | Shimizu et al. ....   | 148/12.1  |
| 2,534,141 | 12/1950 | Morrill et al. ....   | 148/134 X |
| 3,105,780 | 10/1963 | Low.....              | 148/16    |
| 3,239,390 | 3/1966  | Matsukuro et al. .... | 148/12.1  |

### FOREIGN PATENTS OR APPLICATIONS

708,149 4/1965 Canada.....148/16

Primary Examiner—Charles N. Lovell

Attorney—Sughrue, Rothwell, Mion, Zinn & Macpeak

[57]

## ABSTRACT

Process for the manufacture of cold-rolled steel sheets with superior mechanical workability, especially deep-forming qualities, comprising subjecting cold-rolled steel strips to a preliminary annealing step at a temperature below the  $A_1$ -transformation point until the carbon content of said strips is reduced to less than 0.06%, and further subjecting said strips to a second annealing step at a temperature between the  $A_1$ -transformation point and the  $A_3$ -transformation point.

1 Claim, 7 Drawing Figures

PATENTED APR 18 1972

3,657,022

SHEET 1 OF 2

FIG. 2.



FIG. 3.



(A)

FIG. 1.

(B)



(C)



PATENTED APR 18 1972

3,657,022

SHEET 2 OF 2

FIG. 4.



FIG. 5.



FIG. 6.



FIG. 7.



**PROCESS FOR THE MANUFACTURE OF COLD-ROLLED STEEL STRIP WITH SUPERIOR MECHANICAL WORKABILITY, ESPECIALLY DEEP FORMING PROPERTIES**

This application is a continuation of application, Ser. No. 567,334, filed July 20, 1966, now abandoned.

The present invention relates to an improved process for the manufacture of cold-rolled steel sheets with superior mechanical workability, especially deep-pressing qualities.

The main object of the present invention is to provide an improved process of the above kind, for the manufacture rimmed steel base sheet products, yet having a superior deep-forming machinability, in a highly simplified and economical manner.

These and further objects, novel features and advantages will become apparent as the description proceeds in reference to the accompanying drawings, in which:

FIGS. 1 - 7 represents reproduced microscopic photographs,  $\times 100$ , of several examples of structure of steel sheets obtained by the conventional and novel processes.

A conventionally acknowledged measure to improve the press-forming workability of rimmed steel sheets is to reduce the carbon in steel to a reasonable value. The well-acknowledged reason by those skilled in the art is to reduce the quantity of carbide and solid solute carbon in steel, because an excessive amount of these substances in steel will affect upon the steel in hardening thereof upon solidified so that the machinability, especially the press-forming characteristic of the steel products, is considerably affected in the negative sense. When the carbon content is reduced, the carbide in steel will first be reduced and then the solid solute carbon in steel, thereby the steel becoming correspondingly softer, while at the same time the crystal grains are liable to growth. With the growth of the crystal grains, the steel will become still further softer and the crystalline aggregate as a whole will change in its nature in the benefit of improving the deep-machining workability of the steel.

As a commonly employed measure for the reduction of carbon content in steel, the decarburizing annealing process generally known as the open coil process. Generally speaking, the steel sheets prepared and conditioned in this way represents a carbon content of 0.003% or less, thereby showing a highly improved deep-forming workability in comparison with those obtainable in the normally annealed comparative steel products. Even when utilizing this improved process, it is highly difficult, as ascertained from our profound experimental knowledge and experience, to provide steel sheets, capable of representation substantially none of surface defects upon subjected to a deep-pressing deformation, and having rather coarse, yet substantially in an ordered grain size such as, for instance, A.S.T.M.-No. 6, allowable within the limits for the deformation said above.

TABLE 1(a)  
Chemical Composition of Steel Charge

| Charge   | C    | Mn   | P     | S     | O <sub>2</sub> | N <sub>2</sub> |
|----------|------|------|-------|-------|----------------|----------------|
| "A"..... | 0.05 | 0.30 | 0.012 | 0.010 | 0.060          | 0.0010         |

When an example of steel charge "A," briefly to be denoted hereinafter throughout the present specification and having a composition as set forth in the following Table 1(a), was subjected as conventionally, upon solidified, to a coldrolling and a final annealing, the thus obtained sheets provided mechanical properties as enlisted in Table 1 (b), a microscopic photograph of the products being shown in FIG. 1.

In FIG. 1-(a), the results were obtained from the sheet upon annealed in the normal way at 700° C. FIG. 1-(b) and (c) show the results of the sheet upon subjected to a decarburizing annealing at 700° C and 800° C, respectively.

From these results, it can be seen that the mechanical properties of the steel sheets can be appreciably improved by the decarburizing treatment, a considerable amount of finer grains still remains in spite the higher temperature annealing such as, for instance, 800° C, which means that a certain measure is to be adopted for carrying out for letting these finer grains to growth to a maximum allowable limit, so as to improve still further the mechanical properties of the products.

Upon profound experimental and theoretical investigation into the way for improving the growth of crystal grains in the course of the decarburizing annealing of cold-rolled sheet products, it was now found that the mechanism in this sense is decidedly influenced by the existence of minor interlattice particles having particle dimensions in the order of 1 $\mu$  or less and that when the unit number of these minor particles is reduced intentionally, the desired mechanical properties of the sheet products can be substantially improved. As ascertained from experiments, these minor particles are oxides, sulfide or the like, predominantly however the former. Therefore, it may be well expected from the above observation and consideration that by reducing the oxygen content in molten steel to an allowable minimum so as not to adversely affect upon the desirous rimming step, the desired purpose could substantially be fulfilled.

Various different measures for reducing the oxygen content in steel may be conceivable, of which a preferable, economical, easy and simple one may be that which utilizes the balancing condition of oxygen with carbon, manganese or the both. A measure for this purpose is shown in Table 2(a) and 2(b), wherein the carbon content was controlled so as to reduce the oxygen content in steel. The former table specifies an example of steel charge composition, while the latter table enlists the mechanical properties, by way of example, of the steel sheet manufactured therefrom through hot and cold-rolling process

TABLE 2(a).—CHEMICAL COMPOSITION

| Charge   | C    | Mn   | P     | S     | O <sub>2</sub> | N <sub>2</sub> |
|----------|------|------|-------|-------|----------------|----------------|
| "B"..... | 0.12 | 0.40 | 0.015 | 0.021 | 0.029          | 0.0012         |

accompanied by a decarburizing annealing at 750° C. A corresponding microscopic photograph is shown in FIG. 2, as an example. In comparison of these results with those give in the foregoing Table 1(a), it will clearly be acknowledged that in the present example, considerable improvements have been made in the growth of grains. In correspondence thereto, the mechanical properties have been substantially improved

TABLE 2(b).—MECHANICAL PROPERTIES

| Charge   | Yield point, kg./mm. <sup>2</sup> | Tensile strength, kg./mm. <sup>2</sup> | Elongation, percent | Mean value of $\gamma$ | Mean value of Erickson Tests, mm. | C.C.V., mm. |
|----------|-----------------------------------|----------------------------------------|---------------------|------------------------|-----------------------------------|-------------|
| "B"..... | 15.8                              | 28.7                                   | 52.0                | 1.71                   | 12.0                              | 36.6        |

TABLE 1(b)  
Mechanical Properties of Steel Sheet Products

| Charge | Kind of heat treatment    | Yield point, kg./mm. <sup>2</sup> | Tensile strength, kg./mm. <sup>2</sup> | Elongation, percent | Mean value of $\gamma$ | Mean value of Erickson tests, mm. | C.C.V., mm. |
|--------|---------------------------|-----------------------------------|----------------------------------------|---------------------|------------------------|-----------------------------------|-------------|
| "A"    | 700° C. of normal.....    | 26.3                              | 34.0                                   | 47.0                | 1.21                   | 10.5                              | 38.3        |
|        | 700° C. decarburized..... | 22.0                              | 30.7                                   | 51.0                | 1.36                   | 10.9                              | 37.8        |
|        | 800° C. decarburized..... | 18.6                              | 29.8                                   | 51.2                | 1.50                   | 11.5                              | 37.0        |

NOTE.—The thickness of the steel sheet amounted to 0.8 mm.

By adopting the aforementioned improving measure, it could be feared however that in the course of annealing at higher temperature the crystalline grains would become excessively larger or roughened. In FIG. 3, a microscopic photograph taken from the steel sheet having mechanical properties as enlisted in Table 2(b) and conditioned through annealing at 800° C is given. This steel is identified therein by "B" in the similar way as before.

As may be well supposed, this kind of roughened sheet will frequently represent disadvantageous orange-peelings so-called by those skilled in the art, when subjected to severe mechanical fabrication, especially deep pressing job.

The annealing process in the art is commonly carried out in the open coil annealing furnace, in place of the batch type furnace, for improving the processing efficiency and for obtaining a more even distribution of specified temperature. Even in this case, however, part of the coil may frequently elevated locally in its temperature, to such a degree enough to roughen the crystal grains in the corresponding area thus affected. If an improved measure for controlling the crystalline structure so as to create and maintain substantially equally distributed medium size grains in a stabilized manner, the aforementioned way for improving the growing tendency of crystal grains through the way of reducing the aforementioned minor particles in their unit number can be relied upon with safety to a satisfying degree.

We have investigated into the aforementioned phenomenon still further in the above-mentioned direction and brought about an improved process for the manufacture of steel sheets with superior deep-pressing qualities through the way of a higher temperature annealing of the said conditioned steel sheets, yet without any risk of developing excessively coarse or roughened crystal grains.

More specifically to explain, a comparison between the main features of both steels "A" and "B" enlisted in the foregoing Tables 1 and 2, will give the following data:

| Kind of steel | Carbon in steel | Oxygen in steel | Minor particles | Grain growth performance | Mechanical properties | Fear of excessive growth of grains at higher temp. |
|---------------|-----------------|-----------------|-----------------|--------------------------|-----------------------|----------------------------------------------------|
| "A" -----     | 0.05            | 0.060           | Much            | Bad -----                | Better -----          | None.                                              |
| "B" -----     | 0.12            | 0.029           | Small           | Good -----               | Best -----            | Feared.                                            |

In steel "B," it includes twice a high percentage of carbon relative to that contained in steel "A," for the purpose of reducing the said minor particles and thus for improving the performance in grain size growth. As is commonly known, cold-rolled steel sheet products are generally subjected to the open coil annealing for the purpose of realizing a substantially complete decarburizing, it can be said that there would be no practical difference in carbon content between the both kinds of steel "A" and "B," so far as the final products are concerned. Generally speaking, regular decarburizing annealing is carried out at a suitably selected temperature directly below the transition point  $A_1$ . In this case, when the products contain a higher percentage of carbon in steel, a longer extended time period would be necessary to elapse before the termination of a complete decarburizing treatment, while it be allowed to provide a mediumly extended soaking period, the grain size may be subjected to growth substantially to its maximum allowable degree at the specified temperature. Therefore, in this case, the higher carbon content in steel would affect in no direct way upon the grain size as appearing at completion of the annealing treatment.

Now considering such a case wherein the decarburizing is carried out at an intermediate temperature between  $A_1$  and  $A_3$ , there are  $\alpha$ -phase and  $\gamma$ -phase kept in their co-existence in the steel,  $\gamma$ -phase being naturally of austenite, the decarburizing process will progress accompanied by the corresponding reduction of  $\gamma$ -phase, until the carbon content will become a value lower than the solid-soluble limit in the  $\alpha$ -phase specific to the temperature under consideration.

Now taking an example wherein the carbon content in steel is 0.1% and the steel is kept at 800° C for reasonable time period,  $\gamma$ -phase occupying generally in this case about one-fourth the total weight of steel, when the decarburizing treatment is initiated from this condition, the occupation of  $\alpha$ -phase relative to  $\gamma$ -phase will be gradually increased and a considerable reduction of  $\gamma$ -phase or disappearing thereof will occur. Under extreme circumstances it will bring a transfer of grain boundaries formed between  $\alpha$ - and  $\gamma$ -phase, thereby the grain growth in  $\gamma$ -phase being considerably affected with considerable possibilities. Therefore, it can be supposed that at the very moment of disappearing of the  $\gamma$ -phase having a considerably higher carbon content, the expected grain growth will be invited. From observation of FIG. 3 showing coarse or roughened grain sizes which are believed to be caused to take place from a secondary recrystallization, we have supposed with certainty that the extraordinary grain size growth as above referred to substantially depends upon the aforementioned reduction or disappear of the  $\gamma$ -phase. We have further concluded that if this supposition be true, and when steel "B," is beforehand decarburized at a temperature below transformation point  $A_1$ , a decarburizing treatment at an intermediate temperature between  $A_1$  and  $A_3$  could not bring about none of appreciable or excessive degree of grain size growth, or more specifically the disadvantageous roughening. In other words, if the carbon content in the form of  $Fe_3C$  is removed to a satisfying degree at a temperature below transformation point  $A_1$  and then the carburizing treatment is carried out above that point, no abrupt coarsening or size-roughening will take place in any appreciable degree, indeed, in contrast to that case where a so-to-speak straight decarburizing will occur. Because in the former case,  $\gamma$ -phase is already of smaller percentage and thus even through the decarburizing treatment the  $\gamma$ -phase should disappear thereby. FIG. 4 illustrates a microscopic photograph showing the crystalline structure of steel

"B" which has been decarburized at 700° C until the carbon content is reduced to 0.04% and then the decarburizing conditioning is continued at 800° C so as to provide a final carbon content of 0.002% by weight. In this case, as we expected, a decarburizing treatment of the steel at 800° C did not lead to excessive roughening of grain size in any appreciable degree. We have further investigated into the conditioning treatment based upon these data and relative to a large number of steels having various and different compositions in the above sense, and found out that even when the decarburizing treatment is carried out at intermediate temperatures between  $A_1$  and  $A_2$ , while specifying the carbon content at the initiating point of the treatment to 0.03% or less, the disadvantageous coarse grain formation or roughening can be effectively prevented. It should be noted in this case, however, the above specified carbon content of 0.03% is an example of satisfying value for the effective prevention of excessive grain size growth. Therefore, under circumstances a higher carbon content of 0.06% did not invite a roughening of grain size. Based upon the aforementioned experimental data and the analyzed novel teaching, we have ascertained proper treating conditions and the mechanical properties of the final products, the following processing conditions could provide an improved process for the manufacture of thin sheets with superior deep-pressing qualities, said process being realized in such a way that the steel charge is conditioned properly in the course of the steel manufacture so as to favorably affecting the grain growth performance as appearing at the time of later decarburizing annealing, thus prepared molten charge is moulded to steel ingots, which are

hot-rolled, cold-rolled, and then subjected to a decarburizing treatment at a moderate temperature below transformation point  $A_1$ , until the carbon content of steel will be reduced to 0.06% or less, preferably 0.03%.

In the following, several preferred embodiments of the invention will be given only by way of example. For carrying out the process according to this invention, steel charges having a carbon content 0.06 – 0.20%; a manganese content 0.20 – 0.80; least possible contents of P, S and the like, may preferably be used. The contents of carbon and manganese should be so conditioned that the oxygen content in the molten steel be lowest as possible, yet in consideration of the desired rimming action as well as the stabilized working as a whole. In consideration of the balance with the oxygen content, carbon content should preferably be reduced to a reasonable value when manganese content be higher. Recommended hot rolling condition should preferably be 800° – 890° C in terms of finishing temperature. Wind-up temperature may be 550° – 700° C and cold-rolling rate should preferably be 50 – 80%.

#### EXAMPLE 1.

A molten steel charge, named "C," having a composition as set forth in the following Table 3(a) has been prepared, 25 processed as conventionally into ingots.

TABLE 3(a)

|     | C        | Mn | P     | S     | O <sub>2</sub> | N <sub>2</sub> |
|-----|----------|----|-------|-------|----------------|----------------|
| "C" | 0.140.42 |    | 0.010 | 0.016 | 0.027          | 0.0011         |

These ingots were at first hot-rolled at a finishing temperature of 860° C or at a wind-up temperature 570° C, the rolled products being 2.3 mm thick, whereupon the hot-rolled bars were picked and passed through a tandem mill for cold-rolling them to final size of 0.8 mm. The thus produced sheets were decarburizingly annealed under the following conditions, cooled to room temperature and then subjected to a refining rolling by about 10%.

At first stage:

decarburizing anneal at 700° C for 3 hours;

At second stage:

decarburizing anneal at 800° C for 4 hours; subjected to dry soaking at 800° C for 1 hour.

The mechanical properties of the thus obtained cold-rolled sheets are shown in the following Table 3(b), a microscopic photograph of the crystalline structure of a sample taken therefrom, is shown in FIG. 6. When comparing this photograph with that shown in FIG. 5 which illustrates the structure of the same composition of steel, yet subjected to a decarburizing treatment at 750° C, the former represents a highly stabilized and well-distributed crystalline structure, which means a considerable improvement in the art.

TABLE 3(b).—MECHANICAL PROPERTIES

| Charge  | Yielding point, kg./mm. <sup>2</sup> | Tensile strength, kg./mm. <sup>2</sup> | Elongation, percent | Mean value of $\gamma$ | Erickson test, mm. | C.C.V., mm. |
|---------|--------------------------------------|----------------------------------------|---------------------|------------------------|--------------------|-------------|
| C ----- | 15.9                                 | 28.8                                   | 52.3                | 1.75                   | 12.2               | 36.1        |

#### EXAMPLE 2.

A steel charge having a composition set forth in the following Table 4(a) was prepared and processed as before to cold-drawn sheets, 0.8 mm thick.

TABLE 4(a)

#### Chemical Composition

|    |   |        |         |         |                      |                      |                       |
|----|---|--------|---------|---------|----------------------|----------------------|-----------------------|
| 10 | D | C 0.08 | Mn 0.38 | P 0.013 | O <sub>2</sub> 0.018 | N <sub>2</sub> 0.033 | N <sub>2</sub> 0.0011 |
|----|---|--------|---------|---------|----------------------|----------------------|-----------------------|

The thus cold-rolled coils were charged in an annealing furnace, and when the coil temperature reached 500° C, the furnace atmosphere was conditioned so as to show a decarburizing nature, then the temperature was increased to 800° C in the course of 4 hours as the decarburizing process proceeded. At 800° C, a soaking process for further 4 hours was continued, and a dry soaking for an hour, whereupon the products were cooled to room temperature. A refining or conditioning rolling was carried out by about 1.0 %. The mechanical properties of the thus prepared products are shown in the following Table 4(b), while a microscopic photo of the corresponding crystalline structure is shown in FIG. 7.

TABLE 4(b).—CHEMICAL COMPOSITION

| Steel     | Yield point, kg./mm. <sup>2</sup> | Tens. str., kg./mm. <sup>2</sup> | Elongation, percent | Mean value of $\gamma$ | Erick., mm. | C.C.V., mm. |
|-----------|-----------------------------------|----------------------------------|---------------------|------------------------|-------------|-------------|
| "D" ----- | 15.7                              | 28.5                             | 52.2                | 1.72                   | 12.3        | 36.3        |

From the foregoing Examples 1 and 2, it will become clear that according to the present invention, cold-rolled steel sheets having grain size corresponding to A.S.T.M. – No. 6 or 5, superior results substantially equal to, or even more superior results can be obtained, in comparison with those provided by Al-killed steel sheets.

It is to be understood that the above-described examples are only illustrative of the application of the principles of the invention. A number of changes and modifications may be devised by those skilled in the art without departing from the spirit and scope of the invention as set forth in the appended claims.

We claim:

1. Process for the manufacture of cold-rolled steel strip with superior mechanical workability, especially deep-forming properties, comprising the steps of:

- preparing a steel charge including a carbon content of 0.06 to 0.20 wt%, and a manganese content of 0.20 to 0.80 wt %;
- preparing cold-rolled steel strips from said charge through ingot-pouring, hot-rolling and cold-rolling under conventionally employed conditions;
- subjecting said strips to a preliminary annealing at a temperature of 700° C., that temperature being below the  $A_1$ -transformation point to effect decarburization, thus reducing the carbon content of said strips to less than 0.06%; and
- further subjecting said decarburized strips to a second decarburizing annealing at a temperature of 800° C., said temperature being between the  $A_1$ -transformation point and the  $A_3$ -transformation point, thus reducing said strips to the required carbon content, while preventing the formation of a coarsened grain structure.

\* \* \* \* \*